

## UNITED STATES PATENT OFFICE

MARCEL OSWALD, OF NANTERRE, FRANCE, ASSIGNOR TO COMPAGNIE LORRAINE DE CHARBONS POUR L'ELECTRICITE, OF PARIS, FRANCE, A CORPORATION OF FRANCE

## ARC LAMP ELECTRODE

No Drawing. Application filed April 16, 1928, Serial No. 270,580, and in France April 21, 1927.

It is known that electric arcs are considerably stabilized by introducing into the flame of the arc an appropriate mineral material containing metals of low ionization potential. Among them, the alkaline metals and 5 alkaline earth metals, certain metals of the iron group, the metals of the rare earths etc., are much the most employed. Particularly the metals of the rare earths give a white 10 arc flame, slightly bluish, of which the actinic value is very high. This arc is used for this reason for taking pictures in studios and in photogravure.

It has, however, been observed, that these 15 rare earth arcs do not have perfect stability, in that the inevitable fluctuations of the light produce an irregularity in density of the films. It has been possible to remedy this inconvenience somewhat by associating with 20 the rare earths, small quantities of metals with low ionization potential, like calcium, barium or the alkaline metals, but this remedy is not sufficient and the scenic directors instinctively fear that the yellow or orange 25 colour produced by bodies like sodium or calcium spoils the actinic effect.

The invention hereinafter described has for its object to remove all these drawbacks without changing the colour of the arc.

According to the present invention, a perfectly stabilized arc is produced, by introducing into the positive carbon or into the two carbons, small quantities (up to about two per cent) of a refractory reducing material adapted to increase the stability of the 35 arc flame, namely, non-oxidized or slightly oxidized silicon, such as silicon, silicon carbide or silicon oxy-carbide, and the equivalents thereof like boron and zirconium, their 40 non-oxidized or only slightly oxidized compounds, carbides or oxy-carbides.

It has been found that the refractory reducing materials according to the invention are adapted to increase the stability of the arc 45 flame due to their chemical properties, and this by effecting the reduction of the oxy-generated compounds incorporated in the carbons as mineralizers, in the manner described hereinafter, which compounds otherwise produce the disturbing effect above noted due to

their reduction by the carbon in or near the crater of the arc.

The refractory reducing materials according to the invention are incorporated as adjuvants in the already mineralized carbons, 55 which may be mineralized with the rare earths or the alkalies, preferably with compounds of the cerium group. To this end the positive carbon, for example may be cored with a paste containing an organic binding 60 material in solution, or in emulsion in water, and an intimate mixture of silicon, or of one of the compounds mentioned above, with the rare earths of the cerium group, these latter being in the state of oxides, fluorides or 65 oxyfluorides, and also with carbonaceous powders which conveniently dilute the mineral materials. For example, the core hole of this carbon being about one third of the external diameter, the paste will be formed 70 by 50 per cent of carbonaceous materials, 48 to 49 per cent composed of the rare earths, and the remainder by silicon or, preferably, carborundum, which is less expensive and which is more easily obtained in commerce. 75

After mixing the powders intimately, a thick solution of dextrin, gum arabic or any other organic binding material is added so as to finally obtain an extremely thick paste, which is injected under pressure in the carbon tube, in a known manner.

The negative carbon could be formed with an analogous composition, but it has been found experimentally that it is much better to substitute for the rare earths much smaller quantities of potassium carbonate or borate, these salts being capable of being associated with carborundum exactly as for the positive carbon.

Of course the invention is not limited to 90 the examples given above, and consists, in a more general manner, in the incorporation in an arc lamp carbon, such as in the core of the positive or negative carbon, of silicon, boron or zirconium, or a carbide or oxy-carbide of these elements, or compounds of these elements, such as the silicide of boron.

All these materials are associated in a low proportion with a metallic mineralizing element of low ionization potential, this metal- 100

lic element, or the mixture of the said elements being selected according to the desired effect to be obtained.

The said carbons can also be made by introducing a previously hardened homogeneously mineralized rod into a tube of carbon, the union between the homogeneous interior and the tube being effected by means of an adhesive according to well-known methods.

10 The invention also contemplates the introduction of adjuvants like silicon or boron into the shell of carbon, whilst the mineral materials, like the rare earths, are separately introduced into the cores. The results from this method may be favourably compared with those obtained by the method described above. It is nevertheless necessary to take into account in this manner of carrying out the invention, that the proportion of adjuvants may be raised in consequence, because a part is lost by lateral combustion of the carbon before it arrives in the arc.

It should be noted that the term "refractory reducing material adapted to increase the stability of the arc flame", as used in some of the claims herein, is intended to describe and refer to the materials herein described, as producing the improved effects noted, namely, silicon, silicon carbide, silicon oxy-carbide, and the equivalents thereof, with particular reference to boron, boron carbide, zirconium, zirconium carbide, boron silicide, etc. It should also be noted that the term "refractory reducing silicon material", as used in some of the claims herein, is intended to cover and include silicon and non-oxidized or slightly oxidized compounds thereof, with particular reference to silicon carbide and silicon oxy-carbide.

40 It should also be noted that it is essential herein that the materials referred to above should be of a reducing character, that is, that no materials should be used except those which are non-oxygen containing or only slightly oxygen containing, for the following reasons:

(a) The effect is not equivalent when one incorporates in the arc lamp carbons, as adjuvants, already oxidized substances in the one case or refractory reducing substances in the second case, as said carbons already contain important quantities of mineralizing materials, generally in the form of rare earths, and these latter, even if used in the form of commercial fluorides, are not free from oxygen.

(b) When the rare earth oxides are subjected to the action of the arc, a violent reduction by the carbon takes place and a fusible carbide is formed with an ebullition which detaches incandescent particles which are shot off parallelly to the arc and cause fluctuations in the light. This disadvantage subsists when oxidized substances such as silica or boric acid are employed as adjuvants.

(c) On the contrary, when refractory reducing materials like silicon, boron and zirconium, or their carbides, or oxy-carbides, are used, the reduction of the oxidized compounds of the rare earths is effected in the 70 mass of the carbon, in a zone already incandescent but which has not yet reached the crater. The reduction is much less violent and, as it takes place in the mass of the carbon, below the crater, the arc remains perfectly stable.

It should also be noted that it is essential for the effects noted herein, that the silicon, silicon carbide or the like, be employed in very low percentages, not greatly exceeding 80 about two per cent, since it has been found by experiment that the vapourization of these adjuvants adds but few lines to the spectrum of the arc and consequently lowers the luminous output thereof and, therefore, that the percentage incorporated should be kept as low as possible whilst obtaining the desired result. Further, the above limit given has also been found to be necessary in order to avoid too violent a reduction of the rare earth oxides near the crater of the arc.

I claim:—

1. An arc lamp electrode comprising carbon, a mineralizing material including an oxygen-containing metallic compound of low ionization potential, and up to about 2 per cent of a refractory reducing material adapted to increase the stability of the arc flame, intimately mixed together.

2. An arc lamp electrode comprising carbon, an oxygen-containing rare earth compound, and up to about 2 per cent of a refractory reducing material adapted to increase the stability of the arc flame.

3. An arc lamp electrode comprising carbon, an oxygen-containing rare earth compound, and up to about 2 per cent of a refractory reducing silicon material.

4. An arc lamp electrode having a core portion containing carbon, a rare earth oxide, and a refractory reducing material adapted to increase the stability of the arc flame, intimately mixed together, said reducing material being in an amount up to about 2 per cent of the total core material.

5. An arc lamp electrode having a core portion containing carbon, a rare earth oxide, and a refractory reducing silicon material in an amount up to about 2 per cent of the core material, intimately mixed together.

6. An arc lamp electrode having a core portion the diameter of which is about one-third of the external diameter of the carbon and containing carbon and rare earth compounds in about equal proportions and from 1 to 2 per cent of a refractory reducing silicon material.

7. An arc lamp electrode comprising carbon, an oxygen-containing cerium compound,

and up to about 2 per cent of a refractory reducing silicon material.

8. An arc lamp electrode, for use as a negative electrode, comprising carbon, an oxygen-containing alkali metal compound, and up to about 2 per cent of a refractory reducing material adapted to increase the stability of the arc flame.

9. An arc lamp electrode, for use as a negative electrode, comprising carbon, an oxygen-containing potassium salt, and up to about 2 per cent of a refractory reducing silicon material.

In testimony whereof I have hereunto affixed my signature.

MARCEL OSWALD.

20

25

30

35

40

45

50

55

60

65